

# United States Patent [19]

Walz et al.

[11] 3,785,768

[45] Jan. 15, 1974

[54] **PROCESS FOR THE DYEING OF FIBRE MATERIAL CONSISTING OF POLYACRYLONITRILE OR ACRYLONITRILE-CONTAINING COPOLYMERS**

[75] Inventors: Klaus Walz, Leverkusen; Klaus Gerlach, Cologne; Max Schwarz, Berg.-Neukirchen, all of Germany

[73] Assignee: **Bayer Aktiengesellschaft**, Leverkusen, Germany

[22] Filed: Sept. 10, 1971

[21] Appl. No.: 179,571

[30] **Foreign Application Priority Data**

Sept. 11, 1970 Germany..... 2044990

[52] U.S. Cl..... 8/169, 8/84, 8/172, 8/177 AB

[51] Int. Cl. .... D06p 5/06, D06p 3/76

[58] Field of Search ..... 8/84, 172, 177 AB, 8/169

[56] **References Cited**

UNITED STATES PATENTS

2,989,361 6/1961 Hées ..... 8/84 X

|           |        |                    |        |
|-----------|--------|--------------------|--------|
| 2,986,444 | 5/1961 | Rokohl et al. .... | 8/84   |
| 2,145,527 | 1/1939 | Polak et al. ....  | 8/84 X |
| 3,446,569 | 5/1969 | Braun et al. ....  | 8/84   |
| 3,564,630 | 2/1971 | Moussalli ....     | 8/84 X |

*Primary Examiner*—Donald Levy

*Assistant Examiner*—T. J. Herbert, Jr.

*Attorney*—Plumley & Tyner

[57]

## ABSTRACT

Process for dyeing fibre materials consisting of polyacrylonitrile-containing copolymers with cationic dyestuffs in level and deep shades by using as dyeing auxiliaries quaternary ammonium salts which are derived from free ammonium bases of the formula



wherein the R's and A are as defined below.

**4 Claims, No Drawings**

**PROCESS FOR THE DYEING OF FIBRE  
MATERIAL CONSISTING OF  
POLYACRYLONITRILE OR  
ACRYLONITRILE-CONTAINING COPOLYMERS**

The invention relates to a process for the dyeing of fibre materials produced from polyacrylonitrile or acrylonitrile-containing copolymers, with cationic dyestuffs; more particularly it concerns a process for the dyeing of fibre materials produced from polyacrylonitrile or acrylonitrile-containing copolymers, with cationic dyestuffs wherein the dyeing is carried out in the presence of quaternary ammonium salts derived from free ammonium bases of the general formula



in which

$\text{R}$  stands for a  $\text{C}_6\text{-C}_{20}$ -alkyl,  $\text{C}_6\text{-C}_{20}$ -alkenyl or an optionally substituted cycloalkyl or aralkyl radical;

$\text{R}_1$  and  $\text{R}_2$  independently of one another stand for  $\text{C}_1\text{-C}_4$ -alkyl or  $\text{C}_1\text{-C}_4$ -hydroxyalkyl radicals or form together with the nitrogen atom a heterocyclic ring and

$\text{A}$  means an optionally substituted naphthyl or tetrahydronaphthyl radical.

For  $\text{R}$  there may be mentioned by way of example: as alkyl radicals, the n-octyl, 2-ethylhexyl, n-decyl, 2,2-dimethyl-octyl, n-dodecyl, 2,2-dimethyl-decyl, 2-methyl-undecyl, n-tridecyl, 2-methyl-dodecyl, n-tetradecyl, n-hexadecyl and n-octadecyl radicals; as alkenyl radicals, the tetradecenyl, hexadecenyl and octadecenyl radicals;

as cycloalkyl radicals, the cyclohexyl, methyl-cyclohexyl, dimethyl-cyclohexyl, decahydronaphthyl and abietyl radicals;

as aralkyl radicals, the benzyl, chlorobenzyl, phenylethyl, 9(10)-phenyl-stearyl and naphthyl-(1)methyl radicals.

As  $\text{C}_1\text{-C}_4$ -alkyl and hydroxyalkyl radicals for  $\text{R}_1$  and  $\text{R}_2$ , there may be mentioned, by way of example, the methyl, ethyl, propyl, i-propyl, n-butyl, sec.-butyl, 2-hydroxyethyl, 2-hydroxypropyl-(1), 3-hydroxypropyl-(1) and 4-hydroxybutyl-(1) radicals.

Suitable heterocyclic rings which may be formed from  $\text{R}_1$  and  $\text{R}_2$  are primarily the pyrrolidine, piperidine and morpholine rings.

The naphthalene or tetrahydronaphthalene radical may be linked in the 1- or 2-position to the methylene group. However, the naphthalene ring is preferably linked in the 1-position, the tetrahydronaphthalene ring preferably in the 2-position.

Suitable substituents for the naphthalene or tetrahydro-naphthalene radical are, for example,  $\text{C}_1\text{-C}_4$ -alkyl radicals such as the methyl, ethyl, i-propyl or tert.-butyl radicals; furthermore, halogen atoms such as the chlorine or bromine atom; or nitro groups.

Inorganic as well as organic acids are suitable for salt formation with the ammonium bases of the formula (I); preferred acids are the known inorganic acids, such as hydrochloric acid, hydrobromic acid, hydroiodic acid, sulphuric acid, nitric acid or perchloric acid; and organic acids, such as the lower aliphatic carboxylic

acids, e.g., formic acid, acetic acid; aromatic sulphonic acids, such as benzene-sulphonic acid, toluene-sulphonic acid; and the semesters of sulphuric acid, such as methyl-sulphuric acid and ethyl-sulphuric acid.

In the dyeing process according to the invention those quaternary ammonium salts have proved particularly satisfactory which are derived from ammonium bases of the formula (I) in which

10  $\text{R}$  is a  $\text{C}_{10}\text{-C}_{18}$ -alkenyl,  $\text{C}_{10}\text{-C}_{18}$ -alkyl or, preferably, a  $\text{C}_{12}\text{-C}_{18}$ -alkyl radical; and  
 $\text{R}_1$ ,  $\text{R}_2$ , independently of one another, stand for a methyl, ethyl, 2-hydroxyethyl or 2-hydroxypropyl-(1) group.

15 Examples of compounds suitable for the process are the following:

dimethyl-decyl-[naphthyl-(1)-methyl]-ammonium chloride, dimethyl-decyl-[naphthyl-(2)-methyl]-ammonium bromide, dimethyl-dodecyl-[naphthyl-(1)-methyl]-ammonium chloride, dimethyl-tetradecyl-[naphthyl-(1)-methyl]-ammonium chloride, dimethyl-hexadecyl-[naphthyl-(1)methyl]-ammonium bromide, dimethyl-octadecyl-[naphthyl-(1)-methyl]-ammonium chloride, dimethyl-octadecenyl-[naphthyl-(1)-methyl]-ammonium acetate, diethyl-dodecyl-[naphthyl-(1)-methyl]-ammonium iodide, diethyl-dodecyl-[naphthyl-(2)-methyl]-ammonium chloride, diethyl-tetradecyl-[tetrahydronaphthyl-(2)-methyl]-ammonium chloride, dibutyl-octyl-[naphthyl-(1)-methyl]-ammonium bromide, di-(hydroxyethyl)-tetradecyl-[naphthyl-(1)-methyl]-ammonium chloride, di-(hydroxypropyl)-hexadecyl-[naphthyl-(1)-methyl]-ammonium sulphate, hydroxybutyl-methyl-dodecyl-[naphthyl-(1)-methyl]-ammonium methosulphate, di-

30 methyl-abietyl-[naphthyl-(1)-methyl]-ammonium chloride, dibutyl-cyclohexyl-[naphthyl-(1)-methyl]-ammonium bromide, dibutyl-benzyl-[naphthyl-(1)-methyl]-ammonium bromide, diethyl-di-(naphthyl-(1)-methyl)-ammonium chloride, [4-chloronaphthyl-(1)-methyl]-dodecyl-pyrrolidinium chloride and [Naphthyl-(1)-methyl]-dodecyl-piperidinium toluene-sulphonate.

35 The compounds to be used according to the invention can be prepared in known manner, for example, by reacting halomethylated naphthalenes or tetrahydronaphthalene with the appropriate tertiary amines. The reaction may be carried out in the presence of solvents, such as water, alcohols, glycols, formamide, dimethyl formamide, dimethyl sulphoxide or halogenated hydrocarbons, at temperatures from 30° to 150°C.

40 Suitable cationic dyestuffs are dyestuffs from various classes of compounds, for example, diphenyl-methane, triphenylmethane and rhodamine dyestuffs; azo or anthraquinone dyestuffs containing onium groups; furthermore, thiazine, oxazine, methine and azomethine dyestuffs, such as are described, for example, in Ullmanns Encyclopadie der technischen Chemie, Third Edition 1970, Supplement, page 225.

45 The necessary amounts of compounds of the formula (I) to be used according to the invention can easily be determined by preliminary experiments. In general, there are used amounts of about 0.25 to 2.5 percent of these compounds, referred to the weight of the material to be dyed.

50 Suitable acrylonitrile-containing copolymers are, for example, copolymers of acrylonitrile with vinyl chloride, vinylidene chloride, vinyl acetate, vinyl chloroace-

tate, vinyl alcohol, acrylic and methacrylic acid, acrylic and methacrylic acid esters, allyl chloroacetate, or basic vinyl compounds such as vinyl-imidazole, vinyl-benzimidazole, vinyl-pyridine, vinyl-methylpyridine, vinyl-pyrimidine, provided that the proportion of these co-monomers in the copolymers does not amount to more than 20 percent by weight

Dyeing of the polyacrylonitrile fibre materials can be carried out in the usual way, by introducing the material to be dyed into an aqueous dyebath which has been heated to about 50° - 60°C and contains the cationic dyestuff, compounds of the formula (I), added salts, such as sodium acetate or sodium sulphate, and acids, such as acetic acid or formic acid; subsequently raising the temperature of the dyebath to approximately 100°C in the course of about 30 minutes; and then keeping the dyebath at the same temperature until it is exhausted. It is also possible to pretreat the material to be dyed at a temperature of 40° - 100 °C with a liquor which contains the usual salts and acids as well as compounds of the formula (I), but does not contain any dyestuff; to add the dyestuff only then, and to carry out the dyeing at 100°C. Finally, it is also possible immediately to introduce the material to be dyed into a dyebath which contains compounds of the formula (I) and has been heated to approximately 100° C.

With the aid of the process according to the invention it is possible to dye fibre materials which consist of polyacrylonitrile or of acrylonitrile-containing copolymers or contain such polymers or copolymers and which may be present in various stages of processing, for example, as spun cables, combed material, loose material, filaments, yarns, fabrics or knitted fabrics, with outstanding levelness and in deep shades.

Compared with the quaternary ammonium salts commonly used for the dyeing of polyacrylonitrile with cationic dyestuffs, the compounds of the formula (I) have a substantially increased effectiveness which permits of working with substantially smaller amounts of auxiliaries. The increased effectiveness is of particular importance for the dyeing of dyestuffs of high affinity i.e., which draw very fast, since in this case the known retarders have to be used in large amounts, in order to obtain level dyeings.

#### EXAMPLE 1

Yarns of polyacrylonitrile fibres are introduced in a liquor ratio of 1 : 40 into a dyebath which has been heated to 80°C and contains, per litre,

0.1 g of the cationic dyestuff described in Example 8 of British Patent Specification No. 973,259.  
0.25 g sodium acetate  
0.3 g glacial acetic acid and  
0.35 g of the compound of the formula



The bath is heated to 98°C and kept at the same temperature for 60 minutes. A level blue dyeing is obtained.

An equally level blue dyeing was obtained when the dimethyl-dodecyl-(naphthyl-(1)-methyl)-ammonium chloride was replaced with the same amount of one of the following compounds

- a. dimethyl-dodecyl-[naphthyl-(1)-methyl]-ammonium bromide
- b. dimethyl-tetradecyl-[naphthyl-(1)-methyl]-ammonium bromide
- c. diethyl-dodecyl-[naphthyl-(1)-methyl]-ammonium chloride
- d. dimethyl-dodecyl-[naphthyl-(2)methyl]-ammonium chloride
- e. methyl-(2-hydroxyethyl)-octadecyl-[naphthyl-(1)-methyl]-ammonium bromide
- f. bis-(2-hydroxyethyl)-octadecyl-[naphthyl-(1)-methyl]-ammonium chloride
- g. dimethyl-octadecyl-[4-chloronaphthyl-(1)-methyl]-ammonium chloride
- h. diethyl-decyl-[naphthyl-(1)-methyl]-ammonium chloride
- i. N-dodecyl-N-[naphthyl-(1)-methyl]-morpholinium chloride
- j. N-tetradecyl-N-[naphthyl-(1)-methyl]-morpholinium chloride
- k. dibutyl-n-octyl-[naphthyl-(1)-methyl]-ammonium bromide
- l. dimethyl-dodecyl-[naphthyl-(1)-methyl]-ammonium benzene-sulphonate
- m. dimethyl-dodecyl-[tetrahydronaphthyl-(2)-methyl]-ammonium chloride

#### EXAMPLE 2

Yarns of polyacrylonitrile fibres are introduced in a liquor ratio of 1 : 40 into a dyebath which has been heated to 80°C and contains, per litre,

0.1 g of the cationic dyestuff mentioned in Example 1  
0.25 g sodium acetate  
0.3 g glacial acetic acid and  
0.3 g of the compound of the formula



The bath is heated to 98°C and kept at the same temperature for 60 minutes. The bath is then completely exhausted. A blue yarn is obtained which is dyed with outstanding levelness.

A yarn dyed with the same levelness was obtained when the dimethyl-tetradecyl-[naphthyl-(1)-methyl]-ammonium chloride was replaced with the stated amounts of one of the following compounds:

- a. 0.275 g dimethyl-hexadecyl-[naphthyl-(1)-methyl]-ammonium chloride
- b. 0.25 g dimethyl-octadecyl-[naphthyl-(1)-methyl]-ammonium chloride
- c. 0.25 g dimethyl-octadecenyl-[naphthyl-(1)-methyl]-ammonium chloride

#### EXAMPLE 3

Yarns of polyacrylonitrile fibres are introduced in a

liquor ratio of 1 : 40 into a bath which has been heated to 80°C and contains, per litre,

0.1 g of the cationic dyestuff described in Example 1

0.25 g sodium acetate

0.3 g glacial acetic acid

0.35 g of a mixture of the compounds of the formula



and



The bath is gradually heated to 98°C and kept at the same temperature for 60 minutes. A blue dyeing of excellent levelness is obtained.

#### EXAMPLE 4

Yarn of polyacrylonitrile fibres is introduced in a liquor ratio of 1 : 40 into a bath which has been heated to 80°C and contains, per litre

0.04 g of the dyestuff of the formula



0.25 g sodium acetate

0.3 g glacial acetic acid and

0.1 g of the compound of the formula



The bath is heated to 98°C and kept at the same temperature for 60 minutes. A level red dyeing is obtained.

We claim:

1. In the process for dyeing fibers of polymers of acrylonitrile containing at least 80 percent by weight acrylonitrile with cationic dyestuffs the improvement which comprises performing the dyeing in the presence of a dyeing auxiliary which is a quaternary ammonium salt of an ammonium base of the formula:



wherein

20 R is a  $\text{C}_6-\text{C}_{20}$  alkyl or a  $\text{C}_6-\text{C}_{20}$  alkenyl;  $\text{R}_1$  and  $\text{R}_2$ , independently of one another, are  $\text{C}_1-\text{C}_4$  alkyl or  $\text{C}_1-\text{C}_4$  hydroxylalkyl, or a heterocyclic ring when joined together with the nitrogen atom; and  
A is naphthyl, tetrahydronaphthyl, or either of said radicals substituted by  $\text{C}_1-\text{C}_4$  alkyl, halo, or nitro.

25 2. The process of claim 1 wherein  
R stands for a  $\text{C}_{10}-\text{C}_{18}$  alkyl or  $\text{C}_{10}-\text{C}_{18}$  alkenyl radical; and  
 $\text{R}_1$  and  $\text{R}_2$  independently of one another stand for a methyl, ethyl, 2-hydroxyethyl or 2-hydroxypropyl-(1) group.

30 3. The process of claim 1 wherein  
R stands for a  $\text{C}_{12}-\text{C}_{18}$ -alkyl radical, and  
 $\text{R}_1$  and  $\text{R}_2$  stand for a methyl group.

4. Fibre materials of polyacrylonitrile or acrylonitrile-containing copolymers dyed according to claim 1.

\* \* \* \* \*